

## UNITED STATES PATENT OFFICE

2,650,878

METHOD OF PRODUCING ETCHED  
PRINTING PLATES

Mahlon Richard Boyer, Metuchen, and Arthur William Grumbine, Parlin, N. J., assignors to E. I. du Pont de Nemours & Company, Wilmington, Del., a corporation of Delaware

No Drawing. Application December 9, 1949,  
Serial No. 132,200

7 Claims. (Cl. 95—5.7)

**1**  
This invention relates to photography and more particularly to a method of obtaining a resist of gelatin suitable for use in making intaglio printing members. The invention also relates to the preparation of such printing members using the resists.

An object of this invention is to provide improvements in the art of making gelatin resists. A further object is to provide a simple and effective method of making gelatin resists and etched printing members therefrom which can be practiced by the ordinary technician with conventional equipment. Still other objects will be apparent from the following disclosure.

The invention in one of its broader aspects involves exposing a flexible photographic film element having an outer light-sensitive gelatino silver halide emulsion layer and a hydrophobic support through a screen for a suitable time and then through a continuous tone positive, or vice versa. Other conventional types of screens and sequences of exposure can be used. The exposed film is then developed in an aqueous hardening developer solution, e. g., one containing pyrogallol, a small amount of a bisulfite and a relatively large amount of a carbonate whereby the gelatin is tanned at the points of the silver deposits and proportionally to the density of such deposits. The developed film is fixed in a non-hardening fixing bath, washed sufficiently to remove the fixer, bleached in a non-hardening bleach bath containing a water-soluble salt of a metal compound producing an insoluble silver salt image readily soluble in thiosulfate solutions, washed and dried. The bleaching step can be eliminated in a modification of the process just described. The gelatin surface of the film is pressed into contact with a wet surface of a metal printing member, e. g., a copper, aluminum or zinc plate or cylinder, the support removed in some suitable manner leaving the gelatin image-bearing layer firmly adherent to the metal surface. The unhardened gelatin is washed off with hot water leaving a gelatin resist of varying thickness containing silver salts. When the support is a composite one and consists of several layers, e. g., a permanent support, stripping layer and temporary support, the removal requires successive steps.

The surface of the printing plate or cylinder is then etched by treating the gelatin relief image or resist with an acidic solution whereby the image is etched into the surface of the metal. The residue of the hardened gelatin resist is then washed off by a suitable solution, e. g., an

**2**  
aqueous acetic acid solution of moderate to high concentration. Such solutions may also contain a relatively high concentration of sodium chloride.

5 The developed photographic layer can be bleached to form an insoluble silver salt image, e. g., a silver halide, dichromate or ferricyanide image, preferably the latter. The preferred alkali metal ferricyanide bleaching solutions are especially useful when they contain a mixture of borax and boric acid.

10 Various types of photographic film elements may be processed in accordance with the method outlined above but the invention is especially useful with dry-stripping films wherein the gelatino silver halide layer is coated onto a relatively thin permanent support which is in turn adhesively joined to a temporary support by means of a dry-stripping layer. The supports should be 15 made of a hydrophobic material so that the resulting composite element will have good dimensional stability. The permanent support should be readily soluble in commercial solvents so it may be effectively removed from the gelatin layer 20 adhering to the surface of the metal printing member by a simple washing operation. The gelatino silver halide emulsion layer is generally not directly coated onto the film support but first a thin gelatin substratum is applied in order to 25 improve the anchorage.

When a cellulose ester film, e. g., cellulose acetate, cellulose acetate propionate, cellulose acetate butyrate, cellulose nitrate, cellulose propionate, etc., is used in the support for the gelatino silver halide emulsion layer such a support 30 film can readily be removed with commercial solvents for such esters. Mixtures of acetone and ethyl or methyl alcohol and mixtures of acetone and the monomethyl or monoethyl ether of 35 ethylene glycol are especially useful. Acetone can be used alone if desired but because of its high degree of volatility is somewhat difficult to handle. The monoethyl ether of ethylene 40 glycol alone is an excellent single solvent for the permanent support.

The silver ferricyanide, etc., salts which are 45 present in the bleached gelatin layer render a distinct image visible on the metal plate or cylinder. In addition, the salts control the rate and 50 degree of penetration of the etching solution in proportion to the density of the silver salts present and enable one to obtain a good reproduction of the original object field on the surface of the metal plate or cylinder. The silver ferricyanide 55 salts, moreover, seem to have a catalytic effect

## 3

on the etching solution since one can adequately etch copper plates with one concentration of iron perchloride solution in contrast to the five different concentrations which are commonly used.

Fugitive or non-fugitive dyes may be present in the gelatino silver halide layer of the stripping film, if desired, but good results can be obtained with layers free from dyes.

The invention will be further illustrated but is not intended to be limited by the following examples.

## Example I

A photographic stripping film consisting of a cellulose acetate film base bearing on one surface in order a layer of cellulose nitrate, a thin substratum of gelatin and a gelatin backing layer and on the other surface in order a stripping layer composed of a mixture of water-insoluble ethyl cellulose and cellulose nitrate, a cellulose nitrate film, a thin gelatin substratum and a light-sensitive gelatino-silver halide emulsion layer was exposed through a gravure screen (150 line-2:1) for 30 seconds at 10 foot candles and then exposed through a continuous tone positive image for a period of 10 to 30 seconds. The exposed film was then processed as follows:

1. Developed for three minutes at 65° F. in a solution made by mixing 1 part of solution A with 2 parts of solution B.

## A

|                              |        |    |
|------------------------------|--------|----|
| Sodium metabisulfite         | grams  | 10 |
| Methyl-p-aminophenol sulfate | do     | 6  |
| Hydroquinone                 | do     | 3  |
| Pyrogallol                   | do     | 6  |
| Potassium bromide            | do     | 3  |
| Water                        | liters | 1  |

## B

|                  |        |     |
|------------------|--------|-----|
| Sodium carbonate | grams  | 100 |
| Water            | liters | 1   |

2. Rinsed in water at 65° F. for 30 seconds;  
 3. Treated for one minute in an aqueous bath of 10% sodium bisulfite;  
 4. Washed in water at 65° F. for three minutes;  
 5. Fixed for three minutes in 20% sodium thiosulfate solution;  
 6. Washed for five minutes in water at 65° F.;  
 7. Bleached for five minutes in a solution made by admixing the following components:

|                         |       |  |
|-------------------------|-------|--|
|                         | Grams |  |
| Potassium ferri-cyanide | 60    |  |
| Borax                   | 5     |  |
| Boric acid              | 10    |  |
| Water to 1 liter.       |       |  |

8. Washed in water at 65° F. for a period of 15 minutes and then dried at 68° F. at 55% relative humidity.

The gelatin surface of the bleached film was squeegeed into contact with the surface of a wet copper plate. The temporary support which was outermost was then stripped from the cellulose nitrate film support. The latter support was removed by dissolving it in a washing solution composed of 60% acetone and 40% ethyl alcohol. A gelatin relief image which constituted a gelatin "resist" was formed by washing the gelatin layer with water at 125° F. for five minutes. The resist was dried and then treated with 38° Baumé iron perchloride for a period of about 17 minutes, whereby the photographic image was reproduced on the surface of the copper plate. The gelatin residue was washed off the plate after the manner described in Example II.

## 4

## Example II

A photographic stripping film of the kind described in Example I was exposed as described in such example except that a conventional screen having a space to line ratio of 2½:1 was used. The exposed film was then processed and used to make an etched plate by the procedure described in Example I, except that the residue of the relief image was washed off by means of 28% aqueous acetic acid containing a large amount of sodium chloride.

## Example III

A photographic stripping film of the type given in Example I was exposed, developed and washed as described in that example including steps (1) and (2).

3. Fixed for three minutes in 20% sodium thiosulfate solution;  
 4. Washed for five minutes in water at 65° F.;  
 5. Bleached for five minutes in a solution made by admixing the following components:

|                         |       |  |
|-------------------------|-------|--|
|                         | Grams |  |
| Potassium ferri-cyanide | 60    |  |
| Borax                   | 5     |  |
| Boric acid              | 10    |  |
| Water to 1 liter.       |       |  |

6. Washed in water at 65° F. for a period of 15 minutes and then dried at 68° F. at 55% relative humidity.

The gelatin surface of the bleached film was squeegeed into contact with the surface of a wet copper plate. The temporary support which was outermost was then stripped from the cellulose nitrate film support. The latter support was removed by dissolving it in a washing solution composed of 60% acetone and 40% ethyl alcohol. A gelatin relief image which constituted a gelatin "resist" was then made by washing the gelatin layer with water at 125° F. for five minutes. The resist was dried and then treated with 38° Baumé iron perchloride for a period of about 17 minutes, whereby the photographic image was reproduced on the surface of the copper plate. The gelatin residue was washed off the plate after the manner described in Example II.

## Example IV

50 A film of the type given in Example I was exposed and processed to a resist as described in that example except that in place of developing the film in the mixture of solutions A and B it was developed in solution A for two minutes and in solution B for one minute. After the development was completed the film was processed by using steps 3 through 8 of Example I. The gelatin relief image was treated with acid and the copper plate etched and cleaned as described in that example with similar results.

## Example V

65 A film of the type given in Example I was exposed and processed as described in that example except that a fixing bath was used containing 25 grams of boric acid and 250 grams of sodium thiosulfate per liter and after fixing the film was washed and dried, omitting the bleaching step (7) in that example. Etching was accomplished by using a 43° Baumé bath for two minutes, 41° Baumé five minutes, 39° Baumé six minutes and 38° Baumé for six minutes.

70 When brass, aluminum, stainless steel or zinc plates are substituted for the copper plates in

the foregoing examples one obtains similar results.

The invention is not limited to the particular bleach baths of the foregoing examples as other suitable baths which result in a silver ferricyanide or a silver bichromate, etc., image can be substituted. A suitable bath has the following composition:

Potassium ferricyanide \_\_\_\_\_ grams 50  
 Ammonium hydroxide, conc. \_\_\_\_\_ cc 5  
 Water to 1 liter.

Another suitable bleach bath which has a hardening action has the formula:

Potassium bichromate \_\_\_\_\_ grams 20 15  
 Hydrochloric acid, conc. \_\_\_\_\_ cc 10  
 Potassium bromide \_\_\_\_\_ grams 5  
 Water to 1 liter.

Similarly, the invention is not limited to the particular developer solution for developing the silver halide image which is described in Example I. Various other conventional developers can be used with similar results. Changes in contrast, for example, can be accomplished by changing the amount of carbonate in solution B of the developer in Example I. Thus, the amount of sodium carbonate may be varied from 25 to 260 grams per liter. At the lower concentrations the resist is lower in contrast than in Example I and when amounts greater than 100 grams are used the contrast is higher. Potassium carbonate can be used in equivalent amount. The development periods can be varied over a moderate range as apparent to those skilled in the art.

In the washing operation following bleaching when the gelatin relief image or resist is formed the temperature of the water and the time of treatment may vary. Temperatures from 105° F. to 145° F. and times from three minutes to 30 minutes are practical ranges.

Especially good results are obtained with fixing baths which contain material amounts of boric acid, e. g., 15 to 40 grams per liter in addition to the fixing agent.

The etching treatment may be varied depending upon the particular type of metal plate or cylinder used. The etching may be conducted with a single solution or in several solutions of different strength, e. g., iron perchloride solutions varying from Baumé 45° and ending with Baumé 35° can be used. An advantage of the present invention is that a single Baumé iron perchloride solution preferably about 38° can be used instead of the five solutions used by photo-engravers.

In addition to the procedures described above the films may be processed as follows:

1. The film may be exposed, developed in a hardening developer, placed in a stop bath, washed and dried.

2. The film may be exposed, developed in a hardening developer, fixed in a non-hardening fixer, washed and dried.

3. The film may be exposed, developed in a hardening developer, bleached, fixed, washed and dried.

The invention is especially useful in processing the dry stripping films of the types described in copending application Ser. No. 125,198, filed November 3, 1949. It is not limited to such stripping films, however, but can be used with various other types. Suitable additional ones are described in U. S. Patents 2,266,435, 2,275,617 and

2,391,171. Pigments such as iron oxide should be avoided in the films, however, because hardening developers are reduced by them and cause general overall hardening.

The processes of this invention have the advantage that the usual carbon tissues used in the gravure industry can be eliminated with their attendant disadvantages. An important advantage of the invention is that it enables the technician in the gravure art to use one etching solution with the same result previously obtained with several. A further advantage is that the silver salts enable the technician to view the nature of the photographic reproduction before the etching operation is carried out. Still other objects will be apparent to those skilled in the art.

As many widely different embodiments of this invention can be made without departing from the spirit and scope thereof, it is to be understood that the invention is not to be limited except as defined by the claims.

What is claimed is:

1. A process of making an etched printing plate from a dry-stripping film having a gelatino silver halide emulsion layer carried by a thin hydrophobic cellulose derivative support which is adhesively joined to a temporary support by a dry-stripping layer, comprising exposing the emulsion layer separately through a screen and to a photographic picture, developing the exposed film in a hardening developer, fixing said developed film, bleaching the resulting film with an aqueous solution containing a water-soluble alkali metal salt of an acid which forms an insoluble silver salt image readily soluble in thiosulfate solutions, drying the bleached film, pressing the bleached gelatin silver salt layer into contact with the wet surface of a metal printing member, stripping the temporary support from the remaining support, dissolving the latter support, washing the unhardened gelatin from the gelatin layer whereby a relief image is formed and treating the relief image with an acid etching solution whereby an image is etched into the surface of said printing member.

2. A process as set forth in claim 1 wherein the support is dissolved with ethylene glycol monoethyl ether.

3. A process of making an etched printing plate from a dry-stripping film having a gelatino silver halide emulsion layer carried by a thin hydrophobic cellulose derivative support which is adhesively joined to a temporary support by a dry-stripping layer, which comprises exposing the emulsion layer separately through a screen and to a photographic picture, developing the exposed film in a hardening developer, fixing said developed film, bleaching the resulting film with an aqueous solution containing an alkali metal ferricyanide, drying the bleached film, pressing the bleached gelatin silver salt layer into contact with the wet surface of a metal printing member, stripping the temporary support from the remaining support, dissolving the latter support, washing the unhardened gelatin from the gelatin layer whereby a relief image is formed and treating the relief image with an acid etching solution whereby an image is etched into the surface of said printing member.

4. The process of making an etched printing plate from a dry-stripping film having a gelatino silver halide emulsion layer carried by a thin hydrophobic cellulose derivative support which is adhesively joined to a temporary support by a

dry-stripping layer, which comprises exposing the emulsion layer separately through a screen and a photographic image, developing the exposed film in a hardening developer, fixing said developed film, bleaching the resulting film with an aqueous solution containing an alkali metal ferricyanide, borax and boric acid, drying the bleached film, pressing the bleached gelatin silver salt layer into contact with the wet surface of a metal printing member, stripping the temporary support from the remaining support, dissolving the latter support, washing the unhardened gelatin from the gelatin layer whereby a relief image is formed and impregnating the relief image with an iron perchloride solution of 35° to 45° Baumé whereby an image is etched into the surface of said printing member.

5. The process of making a resist from a dry-stripping film having a gelatino silver halide emulsion layer carried by a thin hydrophobic cellulose derivative support which is adhesively joined to a temporary support by a dry-stripping layer, which comprises exposing the emulsion layer separately through a screen and a photographic image, developing the exposed film in a hardening developer, fixing said developed film, bleaching the resulting film with an aqueous solution containing an alkali metal ferricyanide, borax and boric acid, drying the bleached film, pressing the bleached gelatin silver salt layer into contact with the wet surface of a metal printing member, stripping the temporary support from the remaining support, dissolving the latter support and washing the unhardened gelatin from the gelatin layer whereby a relief image is formed.

6. A process of making an etched printing plate from a dry-stripping film having a gelatino silver halide emulsion layer carried by a thin hydrophobic cellulose derivative support which is adhesively joined to a temporary support by a dry-stripping layer, which comprises exposing the emulsion layer separately through a screen and a photographic image, developing the exposed film in a hardening developer, fixing said developed film, bleaching the resulting film with an aqueous solution containing an alkali metal ferricyanide, borax and boric acid, drying the bleached film, pressing the bleached gelatin silver salt layer into contact with the wet surface of a

metal printing member, stripping the temporary support from the remaining support, dissolving the latter support, washing the unhardened gelatin from the gelatin layer whereby a relief image is formed and impregnating the relief image with an iron perchloride solution of 35° to 45° Baumé whereby an image is etched into the surface of the printing member.

7. A process of making an etched printing plate from a dry-stripping film having a gelatino silver halide emulsion layer carried by a thin hydrophobic cellulose derivative support which is adhesively joined to a temporary support by a dry-stripping layer, which comprises exposing the emulsion layer through a screen and to a photographic picture, developing the exposed film in a hardening developer, fixing said developed film, bleaching the resulting film with an aqueous solution containing an alkali metal ferricyanide, borax and boric acid, drying the bleached film, pressing the bleached gelatin silver salt layer into contact with the wet surface of a copper printing member, stripping the temporary support from the remaining support, dissolving the support, washing the unhardened gelatin from the gelatin layer whereby a relief image is formed and impregnating the relief image with an iron perchloride solution of 38° Baumé whereby an image is etched into the surface of the printing member.

MAHLON RICHARD BOYER.  
ARTHUR WILLIAM GRUMBINE.

References Cited in the file of this patent

UNITED STATES PATENTS

| Number    | Name   | Date           |
|-----------|--------|----------------|
| 1,374,853 | John   | Apr. 12, 1921  |
| 1,709,569 | Gorsky | Apr. 16, 1929  |
| 1,926,620 | Herzog | Sept. 12, 1933 |
| 2,100,224 | Snyder | Nov. 23, 1937  |
| 2,207,388 | Kujawa | July 9, 1940   |
| 2,266,435 | Staud  | Dec. 16, 1941  |
| 2,325,519 | Koch   | July 27, 1943  |
| 2,391,171 | Lane   | Dec. 18, 1945  |
| 2,398,056 | Nadeau | Apr. 9, 1946   |

OTHER REFERENCES

Clerc, "Photography," 2nd edition, 1937, Pitman & Sons, page 278.